

# UNITED STATES PATENT OFFICE.

SAMUEL E. SHEPPARD, OF ROCHESTER, NEW YORK, ASSIGNOR TO EASTMAN KODAK COMPANY, OF ROCHESTER, NEW YORK, A CORPORATION OF NEW YORK.

## PURIFYING AND WASHING PROCESS.

1,357,733.

Specification of Letters Patent.

Patented Nov. 2, 1920.

No Drawing.

Application filed June 5, 1918. Serial No. 238,400.

To all whom it may concern:

Be it known that I, SAMUEL E. SHEPPARD, a subject of the King of Great Britain, residing at Rochester, in the county of Monroe and State of New York, have invented certain new and useful Improvements in Purifying and Washing Processes, of which the following is a full, clear, and exact specification.

10 This invention relates to the washing and purifying of cellulose esters and it finds its most important application in the treatment of cellulose nitrate to remove the unfixed acid and unstable acid compounds which are 15 associated therewith.

The objects of my invention are to effect this purification and washing more thoroughly, in shorter time, using less water, and less space than in prior processes; to utilize 20 cheap ingredients which can be used repeatedly; to employ a solution of a salt derived from a strong base and a strong acid whenever the process requires a non-hydrolyzable salt; to employ a saline leach of 25 sufficient strength to osmotically compress the treated material and extract water, acid, and unstable acid compounds therefrom while depressing the dissociation of these acid substances as well as the stable esters; 30 to utilize soft water for washing as well as hard water; to provide a process which will be effective at ordinary or room temperatures yet may be usefully combined with heating operations; to obtain these advantages 35 without decomposing the relatively stable esters which are undergoing treatment; and to obtain a product which shall be, when necessary, practically, free from particles of insoluble opaque mineral matter. Other objects will hereinafter appear.

Since my invention at present finds its widest application in the purification of nitrated cellulose fiber I shall describe its application to that material, by way of illustration. As is well known, the cellulose, usually cotton, is nitrated in a bath of concentrated nitric and sulfuric acids. When nitration has progressed to the desired degree, the mixture is subjected to a centrifuging action to wring out as much acid as possible. It is then plunged, "drowned" or "soused" in a bath of water to remove some of the acid, keep the mass cool, and prepare it for the subsequent purification operations.

55 The unpurified nitrated cellulose at this

stage of the process consists of fibers or fibrous fragments composed of the higher and relatively stable cellulose nitrates together with adherent or mechanically held acid and capillary retained or adsorbed acid. There may be present also unstable so-called "lower" cellulose nitrates together with some cellulose sulfate or cellulose-sulfuric-acid and it is probable these contain part of the adsorbed acid. In order to make 60 the final product stable and for other reasons, it has been long desired to eliminate all other of these substances except the higher relatively stable cellulose nitrates. It has been attempted to remove these impurities 65 by prolonged washing in successive changes of water or successive boilings in different changes of water, either of these methods being at times supplemented by pulping and treatment with a dilute alkaline bath to neutralize any acid that may still remain. Such processes, although widely used, have been 70 open to several objections. The amount of water used has been very great; the time of the operations has been prolonged, thus keeping a large mass of material under various stages of treatment in the factory and requiring a relatively large space and equipment; and my experiments show that the 75 elimination of the impurities has not always 80 been as complete as was believed. Furthermore, hard water or water containing mineral substances which give it a mild alkaline reaction was generally thought to be necessary for washing because of its possible 85 neutralizing properties. The known methods have the additional disadvantage that the prolonged washing, boiling or neutralizing operations tend to partially defeat 90 their own object by causing a decomposition 95 of the relatively stable cellulose nitrates which are being purified.

I have discovered that if the substances to be purified are treated with a strong leach of a nearly neutral saline solution, preferably 100 nearly saturated, and then washed, there will be removed from 50 to 100 per cent. more unfixed acid than is removed by plain washing in soft water. Also the purification can be effected in  $\frac{1}{10}$  to  $\frac{1}{4}$  of the time 105 whatever the nature of the water. Moreover, the number of changes of water is greatly reduced; so that less water, space and apparatus are required for a given output and soft water may be used as well as 110

hard. Furthermore, the relatively stable cellulose nitrates are practically unaffected by my treatment. Moreover my process may be combined with the known boiling methods with a substantial reduction of the washing periods between boilings. Furthermore the saline leach can be used as a semi-stabilizing stop bath so that boiling may be taken up at any desired time after nitrating.

10 In one form of my invention, which I cite by way of a specific illustration, the soused nitrated cotton is wrung in a centrifugal machine for twenty minutes while being sprayed with a nearly saturated and nearly 75 neutral solution of sodium sulfate. It is then removed to a bath of similar strong sodium sulfate solution and leached for one hour. Next it is wrung and drained between 80 squeeze rolls or in a centrifugal for fifteen 85 minutes. These operations of leaching in successive baths and wringing and draining off the solution between baths are then repeated; so that in a typical case the cotton will receive a total of four or five sulfate 90 leachings of one hour each. During any of these leaching operations the baths may be warmed to accelerate the action, a convenient temperature being 35° C. However, room temperature is generally adequate.

95 15 Furthermore, I may sometimes (but not necessarily) make one of the leaching baths, preferably one of the intermediate baths, mildly alkaline by adding small quantities of sodium carbonate. This will reach and 100 neutralize acid that may be contained in the interior of balls or clumps of the cotton. The subsequent wringing and leaching steps remove any remaining carbonates along with the other substances which are leached 105 out. The purified nitrated cotton is finally washed, for instance by simultaneously wringing in a centrifugal machine and spraying with water for fifteen or twenty minutes, the sulfate being thoroughly removed. The whole process from sousing to 110 final washing does not require more than half a day as compared with one or two weeks' treatment in the usual washing processes other than boiling methods and is, therefore, adapted to large scale work.

115 15 Wringing operations between leachings are sometimes inconvenient, requiring as they do centrifugals, rolls or other machinery and are not indispensable. I may, for example, transfer the nitrated cotton directly from the sousing bath to a nearly 120 saturated, practically neutral, sodium sulfate leaching solution, where it remains for an hour. The solution is next removed by 125 natural bottom drainage for a half hour and fresh leaching solution then poured onto the cotton. These leaching periods in strong sulfate solutions and intermediate gravity draining periods are repeated, say seven 130 times, when the nitrated cotton is thor-

oughly washed. In this form of my invention the action may also be hastened, if desired, by warming the leaching baths to about 35° C., the precise temperature being unimportant. When, as in this case, no 70 wringing is used between leachings, it is preferable to make one of the baths, say the sixth, mildly alkaline with small amounts of sodium carbonate. This process does not take over twelve or fifteen hours, particularly if a centrifugal and water spray 75 be available for the final removal of the sulfate from the cotton. With hard water of permissible alkalinity the same total acid may be removed, but it requires much more 80 water, many more changes, and therefore greatly prolonged treatment as compared with my method.

85 As regards the particular neutral leaching solution, I prefer a nearly saturated solution of sodium sulfate because it has the necessary properties and is at the same time a cheap by-product from the manufacture of nitric acid. If the commercial sodium sulfate contains free acid, it is easy and inexpensive to neutralize it.

90 Moreover, the used leaching solution may be treated to neutralize the acid which it has extracted and then can be employed again. I may add, for example, comminuted 95 calcium carbonate and filter, thereby regenerating the bath. I find that this neutralizes the acid substances without, however, making the bath too alkaline. It becomes practically neutral, in fact, its alkalinity being very small and comparable to that of hard water. It is especially noted 100 that this regeneration requires no analysis or titrations by skilled persons but unskilled labor may be employed. This regeneration of each bath may be repeated 105 indefinitely.

110 I prefer a salt, like sodium sulfate, derived from the union of a strong base with a strong acid because such a salt gives a 115 substantially neutral solution and does not hydrolyze to make the solution alkaline or acid, as is the case when a weak acid is combined with a strong base or a weak base combined with a strong acid. The initial neutrality of the leaching solution reduces any tendency to decomposition of the relatively stable esters.

120 The leaching step is ordinarily carried out at normal or room temperatures and pressures. In some cases, however, as above indicated, I may heat the leaching bath to accelerate the action or I may heat the water used in the subsequent washing. Because the strong leaching bath tends to prevent 125 the ionization of the treated materials, the effect of heating will be less injurious than where boiling takes place in water alone.

130 As a further modification I may agitate the material which is undergoing treatment

by air under pressure, or such agitation may take place just prior to or subsequent to a leaching operation.

From the physical-chemistry standpoint it appears that the remarkable action which takes place in the leaching steps may be explained as follows:

The "acid" nitrocellulose consists of fibers or fiber fragments containing inner filamentous canals, the aggregate of fibers having a very large surface in proportion to its mass. The material of the fibers consists of the stable cellulose esters and some less altered cellulose carrying both adherent 15 or mechanically held acid and adsorbed acid. The adsorbed acid is probably loosely combined in an ionizable and readily hydrolyzable complex with hydrated cellulose residues which exist as a 20 membrane at the surface of the fibers. All these substances tend to a definite equilibrium in respect of acid residue under given conditions of temperature, concentration, etc., and this equilibrium is quite different 25 in water than when my saline leach is employed. The adherent acid and the adsorbed acid will come to equilibrium relatively rapidly, whereas adjustment is slow between the adsorbed acid and the 30 stable esters. In the prolonged boiling and neutralizing steps of the prior art the equilibrium between the stable esters and the unfixed acids is liable to be altered in such a direction that considerable quantities of 35 the stable esters tend to decompose.

In my process, however, the removal of the adherent and adsorbed acids is effected osmotically without injuriously affecting the equilibrium between the stable esters 40 and the unfixed acids, this effect being due in part to the isohydric depression of the dissociation (of ionization and swelling) of the adherent acid and of the adsorbed acid substances by the mass action of the 45 concentrated neutral salt. The osmotic action produces a powerful contraction of the osmotic cells and membranes constituted by the fibers and fiber fragments, which contraction is an aid in removing any 50 acid held by the fiber. This also tends to check decomposition of the true cellulose esters.

Of course a correct knowledge of the physico-chemical theory of my process is 55 not indispensable to its practical application, but it gives an insight into how I obtain the new results which differ from the prior art, particularly those processes which employ so-called stabilizers.

The action of my leaching bath is independent of the degree to which the nitration has been carried out, if said degree be within the limits of commercial practice. The presence of unaltered cellulose is also 65 immaterial in the purification steps.

Nitrocellulose treated according to my method is more quiet in the burning test than the average nitrocellulose obtained by prolonged washing alone. It dries without trouble at the usual temperature; is 70 soluble in the acetone-methyl alcohol mixture and gives a viscosity at least equal to and generally better than that of similar products in the prior art. The product is 75 freer from opaque mineral matters which are sometimes introduced into the film by prolonged washing with hard waters. This freedom from opaque particles is particularly important where the nitrocellulose is to be worked up into transparent films for 80 photographic purposes.

While it is generally preferred to wash out the (residue of) leaching salt remaining after the free acid is removed, yet in some instances even this additional operation is 85 unnecessary or may be much abbreviated, because the presence of the salt is harmless in many of the compositions into which nitrocellulose enters and adds to the stability. 90

I have described my invention as applied to the removal of the acid impurities from nitrocellulose by way of illustration but my research has shown that it is also applicable to the removal of the unfixed acid and acid 95 substances which remain after esterification when making analogous material under similar conditions. I also note that my process can be used equally well whether the original cellulose which was nitrated 100 was derived from cotton, wood, paper or any usual or preferred source.

While a plurality of leachings are generally advisable, one such leaching in strong salt solution will greatly shorten the time 105 of subsequent washing and removal of acid. I may also alternate leaching operations with washing steps instead of mere draining steps in order to accentuate the alternate osmotic compression and hydration. 110

Having thus described my invention what I claim and desire to secure by Letters Patent of the United States is:

1. The process of removing unfixed acid and acid substances from bodies of cellulose esters having large surface in proportion to their mass, which includes the steps of treating the same with a strong solution of a salt and then washing out said salt therefrom while said bodies remain in a 120 substantially undissolved state.

2. The process of removing unfixed acid and acid substances from bodies of cellulose esters having large surface in proportion to their mass, which includes the steps of treating the same with a strong, nearly neutral solution of a salt and washing the same while said bodies remain in a substantially undissolved state. 125

3. The process of removing unfixed acid 130

and acid substances from bodies of cellulose esters having large surface in proportion to their mass, which includes the step of treating the same with a strong solution of 5 sodium sulfate.

4. The process of removing unfixed acid and acid substances from bodies of cellulose esters having large surface in proportion to their mass, which includes the step of 10 repeatedly treating the same with a strong solution of a salt while said bodies remain in a substantially undissolved state.

5. The process of removing unfixed acid and acid substances from nitrated cellulose, 15 which includes the steps of treating the same with a strong, nearly neutral solution of a salt and washing the same while said bodies remain in a substantially undissolved state.

20 6. The process of removing unfixed acid and acid substances from nitrated cellulose, which includes the step of treating the same with a strong solution of a salt formed from a strong base and a strong acid and finally 25 washing the same while said nitrated cellulose remains in a substantially undissolved state.

7. The process of removing unfixed acid and acid substances from nitrated cellulose, 30 which includes the step of treating the same with a strong solution of sodium sulfate.

8. The process of removing unfixed acid and acid substances from nitrated cellulose, 35 which includes the steps of treating the same with a strong, nearly neutral solution of sodium sulfate and washing the same.

40 9. The process of removing unfixed acid and acid substances from nitrated cellulose, which includes the steps of treating the same in a nearly saturated solution of sodium sulfate and washing the same with water.

10. The process of removing unfixed acid and acid substances from bodies of cellulose esters having large surface in proportion to 45 their mass, which includes the steps of alternately treating the same with strong salt solution and draining such solution therefrom.

50 11. The process of removing unfixed acid and acid substances from bodies of cellulose esters having large surface in proportion to their mass, which includes the steps of treating the same with a strong solution of a salt, removing a large part of such solution from said bodies by subjecting them to pressure and finally washing the same while said bodies remain in a substantially undissolved state.

60 12. The process of removing unfixed acid and acid substances from nitrated cellulose, which comprises treating the same repeatedly with a strong solution of sodium sulfate.

65 13. The process of removing unfixed acid and acid substances from nitrated cellulose,

which comprises soaking the same in a strong solution of sodium sulfate and draining such solution therefrom.

14. The process of removing unfixed acid and acid substances from nitrated cellulose, 70 which comprises repeatedly subjecting the same to treatment with strong sodium sulfate solution and removing a large part of such solution between each treatment and finally washing the same. 75

15. The process of removing unfixed acid and acid substances from nitrated cellulose, which comprises the steps of successively treating the same to the action of strong sodium sulfate solution, during the intervals 80 between said successive treatments, removing a large part of said solution by pressure, and finally washing out said solution while keeping said nitrocellulose under pressure.

16. The process of removing unfixed acid and acid substances from nitrated cellulose, which includes the step of treating the same with warm strong sodium sulfate solution.

17. The process of removing unfixed acid and acid substances from nitrated cellulose, 90 which includes the steps of treating the same successively to a plurality of baths of strong salt solution, one of said baths being mildly alkaline, and others substantially neutral.

18. The process of removing unfixed acid and acid substances from bodies of cellulose esters having large surface in proportion to the mass, which comprises repeatedly treating the same with strong salt solution, and repeatedly neutralizing the acid and acid 100 substances taken up during said treatments by said solution.

19. The process of removing unfixed acid and acid substances from nitrated cellulose, which comprises treating successive batches 105 of said nitrated cellulose with a strong sodium sulfate solution, and neutralizing the acids and acid substances taken up by the solution during said treatments by adding calcium carbonate to said solution and filtering the same between said treatments.

20. The process of removing unfixed acid and acid substances from bodies of cellulose esters having large surface in proportion to their mass, which includes soaking the 115 same in a strong solution of a salt formed from a strong base and a strong acid and finally washing out said salt therefrom while said bodies remain in a substantially undissolved state. 120

21. The process of removing adherent and adsorbed acid and acid substances from organic compounds which have large surface in proportion to mass, said surface comprising osmotic membranes, which includes the 125 steps of leaching said compound in a saline bath sufficiently concentrated to osmotically compress the material and extract water and unfixed acids while isohydrically depressing the dissociation of the compounds, and 130

finally washing the same while said compounds remain in a substantially undissolved state.

22. The process of removing unfixed acid and acid substances from bodies of cellulose esters having large surface in proportion to their mass, which includes the steps of treating the same in a strong salt solution, and wringing and washing the same while said bodies remain in a substantially undissolved state.

23. The process of treating soused nitrated cellulose, which includes the steps of simultaneously wringing said nitrated cellulose and washing the same with a strong salt solution.

24. The process which comprises sousing nitrated cotton, wringing said nitrated cotton and washing it with a strong salt solution, leaching said nitrated cotton in a bath of strong salt solution, wringing and drain-

ing said solution from said nitrated cotton, repeating said leaching, wringing and draining operations, and finally washing and wringing said nitrated cotton.

25

25. The process which comprises, sousing nitrated cotton, wringing said nitrated cotton while spraying the same with a strong sodium sulfate solution, leaching said nitrated cotton in a strong sodium sulfate solution, wringing said solution from said nitrated cotton, repeating said leaching and wringing operations alternately, the solution being warmed during certain of said leaching operations, and said solution during one of said leaching operations being mildly alkaline, and finally wringing and spraying said nitrated cotton with water.

Signed at Rochester, New York, this 27th day of May, 1918.

SAMUEL E. SHEPPARD.